

Patented May 16, 1939

2,158,184

# UNITED STATES PATENT OFFICE

2,158,184

## TONING AND INTENSIFYING SOLUTIONS

**Kenneth C. D. Hickman and John C. Hecker,  
Rochester, N. Y., assignors, by mesne assign-  
ments, to Eastman Kodak Company, Jersey  
City, N. J., a corporation of New Jersey**

No Drawing. Application April 27, 1934, Serial  
No. 722,730. Renewed March 12, 1938

5 Claims. (Cl. 95—88)

This invention relates to toning and intensifying solutions for developed photographic images, whether in the form of negatives or prints, and more particularly to a new type of single solution toning and intensifying bath.

As is well known, silver salts will react with other soluble salts, but metallic silver is attacked most readily by elementary substances or their equivalents. It is for this reason that one of the best known methods of sulfide toning involves first, the conversion of the metallic silver to a salt, such as silver bromide, by treatment with a mixture of potassium bromide and potassium ferricyanide and, second, the conversion of the silver bromide to silver sulfide by double decomposition with sodium sulfide. This particular conversion, however, cannot be made in one stage in a single solution because the ferricyanide attacks the sodium sulfide more readily than the silver. The problem is then to find an oxidizing agent sufficiently powerful to oxidize the silver and yet be compatible with the sulfiding agent. A number of single solution sulfide toning processes have been developed to solve this problem, but each suffers some drawback. In the well known hypo-alum process, for example, the bath draws sulfur from the hypo and oxidizer from the air, but the solution must be heated and the process is slow. Other sulfide toning baths comprising sodium or barium sulfide and sodium meta-nitro-benzene sulfonate are slow in action and vile in odor.

It is the principal object of the present invention to provide a single solution toning bath which will meet many of the requirements of such baths without at the same time possessing the limitations of the hitherto known solutions. A further object is to provide a single solution bath which may not only be used for toning the image, but also for intensification. A still further object is to provide a bath of this type possessing the novel property that it may be employed for toning a photographic image immediately after development and before fixing. With the above and other objects in view which will become apparent as the description proceeds, we have set forth our invention in the following specification and examples which are included merely for purposes of illustration and not as a limitation thereof.

We have discovered that various thio-compounds or their derivatives notably the soluble thiosulfates, the trithionates and tetrathionates may be employed for the toning and intensification of silver images. These thio-compounds, although sometimes grouped in separate classes in the chemical text books, may, for the purposes of this invention, be grouped in one class, because they all contain available sulfur in its di-va-lent condition. Many other substances contain di-

valent sulfur, mostly the thioureas and the polysulfides, but in these cases the di-va-lent sulfur is connected to an unlike atom or to another unsaturated sulfur atom. The di-va-lent sulfur in the class of compounds considered within the scope of this invention is connected by one or two bonds to another sulfur atom, which latter atom is otherwise fully oxygenated and is in its hexa-va-lent condition. We shall find it convenient first briefly to discuss the trithionates and tetrathionates after which we shall discuss the thiosulfate derivatives, in particular the compounds of thiosulfuric acid and organic substances containing a quinone or hydroquinone grouping. In these discussions we shall refer to some of the broader theoretical aspects of our discovery, although we are not to be understood as in any way limiting our invention thereby.

We have found that the silver salts of all three classes of compounds readily eliminate silver sulfide and that the trithionates and tetrathionates are particularly valuable in our invention because they are stable in the presence of acid and mild oxidizing agents. This is of especial importance, since in order to be suitable for use in a toning solution, the toning agent must be of the kind which will produce a silver salt which will readily decompose into silver sulfide as fast as the metallic silver is oxidized, as otherwise the image will wander or suffer reduction. Although neutral permanganate or permanganate-phosphate admixtures with the thionates form somewhat reducing baths, which are, nevertheless, quite operative for the purposes of our invention, ferric salts, such as ferric sulfate, and the above mentioned thionates, give conversion to sulfide with only a slight loss. Typical toning solutions produced from the thionates according to one form of our invention are given below:

### (Trithionate)

|                       |       |      |
|-----------------------|-------|------|
| Water                 | c. c. | 100  |
| Ferric sulfate        | g.    | 1 45 |
| Sulphuric acid        | c. c. | 0.25 |
| Potassium trithionate | g.    | 1.5  |

### (Tetrathionate)

|                         |       |      |
|-------------------------|-------|------|
| Water                   | c. c. | 100  |
| Ferric sulfate          | g.    | 1 50 |
| Sulphuric acid          | c. c. | 0.25 |
| Potassium tetrathionate | g.    | 1.5  |

### (Tetrathionate)

|                          |       |       |
|--------------------------|-------|-------|
| Water                    | c. c. | 100   |
| Potassium permanganate   | g.    | 1 .55 |
| Di-sodium acid phosphate | g.    | 8.8   |
| Potassium tetrathionate  | g.    | 1.0   |

While in the above description and examples of the thionates we have referred for convenience

to their potassium salts, we may employ them in the form of the sodium, rubidium, caesium, ammonium, calcium and the like compounds. In fact, almost any soluble thionate may be employed with equal facility according to our invention.

The tones produced by the above solutions are an unattractive yellow, but the images are light sensitive and can be intensified, if desired, by treatment with solutions of double silver nitrite or sulfite, as described for example in the Journal of the Franklin Institute for 1933, vol. 216, pages 59, 627, 683, and 706, the first loss on toning being thus more than recovered.

We come now to consideration of the thiosulfates as sulfiding agents or as sources of labile sulfur. One of the few oxidizing agents that thiosulfates such as hypo will tolerate (though only for a short time) is ferricyanic acid, conveniently in the form of the potassium salt. A mixture of hypo and potassium ferricyanide, as ordinarily compounded, is, however, not a sulfiding agent, but an almost perfect solvent for the silver image, constituting in fact, the well-known "Farmer's reducer." This is because the silver thiosulfate first produced is dissolved by the excess thiosulfate before it has time to eliminate silver sulfide. We have discovered that if the relative proportions of the hypo and ferricyanide are reversed, a weak sulfide toner is produced, some of the silver in each density being converted to sulfide before the more usual reduction process has operated. Further to emphasize this important point, we give, side by side, the well-known reducing recipe and a toning bath coming within the scope of our invention.

|                             | Farmer's reducer | Parts by weight | Sulfide toner |
|-----------------------------|------------------|-----------------|---------------|
| 40                          |                  |                 |               |
| Potassium ferricyanide..... |                  | 1               | Parts 5-10    |
| Hypo.....                   | 20               |                 | .1-1.0        |
| Water.....                  | 100              |                 | 100           |

Such a toning bath as the right-hand one above, which is applicable to special processes, is not of general usefulness because of its short life and incomplete action. We have, however, made the fortunate discovery that certain organic thiosulfuric acid derivatives possess at one and the same time a greater stability toward acid and oxidizing agents and a greater instability toward silver so that their silver salts, which are more easily formed, are also more easily broken up, depositing silver sulfide. Such derivatives may be employed as toners with excellent results.

Among these derivatives may be mentioned the quinone and hydroquinone derivatives of thiosulfuric acid. Of the hydroquinone compounds, hydroquinone monothiosulfuric acid, hydroquinone dithiosulfuric acid and hydroquinone tetra-thiosulfuric acid may all be formed by the reaction of a thiosulfate and quinone under controlled conditions. The conditions are not difficult to obtain and the acids are all easily prepared; the "mono" form resulting from dropping quinone dissolved in dilute acetic acid into ordinary hypo, the "di" form by adding hypo to quinone in acetic acid, while the "tetra" form separates in almost theoretical yield when solutions of chromic acid and hypo are added simultaneously to a solution of quinone in acetic acid. These three hydroquinone thiosulfuric acids are

considered to have the following structural formulae:



It will be seen that each acid contains sulfur in the condition specified above as important to this invention, namely, attached to another fully oxygenated sulfur atom.

To form a toning bath, the hydroquinone compounds must be oxidized to the quinone form, or must be mixed with quinones or other oxidizing agents. Suitable oxidizing constituents of a toning bath, by way of example, are ordinary (benzo) quinone or potassium dichromate and an excellent toning bath for bromide and other developing out papers according to our invention, has the following composition:

|                                          |           |        |
|------------------------------------------|-----------|--------|
| Hydroquinone tetrathiosulfuric acid..... | g.....    | .5     |
| Quinone.....                             | g.....    | 1.0    |
| Sulfuric acid.....                       | c. c..... | .25    |
| Water.....                               | c. c..... | 100.00 |

The above bath can be used continuously until the concentration of hydroquinone produced in the toning reaction becomes so high that an equilibrium mixture results which is non-reactive. The activity of the bath can then be restored, by adding chromic acid, although the rejuvenated bath stains slightly from dyes produced by secondary oxidation.

A toning bath containing as much as 1 per cent of free mineral acid may have a somewhat harmful effect on gelatine emulsions and films and prints to be intensified in such a bath should be fixed in hypo containing alum and the toning solution should likewise be loaded with alum. Bearing in mind that hydroquinone is a product of the toning reaction, the toning solution in use may contain, in accordance with our invention, a quinone thiosulfuric acid, a hydroquinone, a mineral acid, and an alum, for example, chrome alum, potassium chromium sulfate. Such a solution containing chiefly the mono- and di-thiosulfuric acids, which confer both toning and intensifying properties may be made by mixing hydroquinone, chromic acid, and hypo, chemicals which are readily available in the photographic laboratory. Inasmuch as the toning solution does not keep well, its constituents should be bottled separately, a convenient recipe being as follows:

|                            |           |     |
|----------------------------|-----------|-----|
| Solution A                 |           |     |
| Water.....                 | c. c..... | 500 |
| Potassium dichromate.....  | g.....    | 16  |
| Sulfuric acid (conc.)..... | g.....    | 17  |
|                            |           | 75  |

|                  |       |     |
|------------------|-------|-----|
| Solution B       |       |     |
| Water            | c. c. | 500 |
| Hydroquinone     | g.    | 16  |
| Sodium bisulfite | g.    | .75 |
| 5 Solution C     |       |     |
| Water            | c. c. | 500 |
| Hypo             | g.    | 11  |
| 10 Solution C'   |       |     |
| Water            | c. c. | 350 |
| Hypo             | g.    | 80  |

Equal portions of the first three solutions are employed, B being poured into A in a thin stream with rapid stirring, after which C is added to the mixture, also with stirring. The resulting solution is then cooled down to below 70° F. for use.

If a quicker bath is needed, one tenth the volume of Solution C' may replace Solution C. A very vigorous bath may, for example, have the following formula:

|                                  |       |       |
|----------------------------------|-------|-------|
| Hydroquinone dithiosulfuric acid | g.    | .5    |
| Quinone                          | g.    | 1.0   |
| Sulfuric acid                    | g.    | .25   |
| 25 Water                         | c. c. | 100.0 |

This solution should be used at about 65-75° F. An example of a toning bath containing hydroquinone monothiosulfuric acid has the following

30 composition:

|                                                                                        |       |      |
|----------------------------------------------------------------------------------------|-------|------|
| Quinone                                                                                | g.    | 1.0  |
| Water                                                                                  | c. c. | 100  |
| Sulfuric acid                                                                          | c. c. | 0.25 |
| 35 Hydroquinone monothiosulfuric acid (conveniently in the form of its potassium salt) | g.    | 0.5  |

This toning solution produces a reddish-purple tone which can be varied by varying the quantity 40 of the hydroquinone salt as desired.

While we do not wish to confine ourselves to any particular theory or explanation of the mechanism involved in the various reactions in toning by means of these hydroquinone thiosulfuric acids, we believe that the first product of toning 45 is not silver sulfide, but a silver hydroquinone thiosulfate, for example, silver hydroquinone dithiosulfate in the case of a solution such as indicated in the preceding paragraph. This salt 50 is creamy white and very insoluble, but in the presence of the excess oxidizing agent and acid soon changes to a greenish black. This compound which constitutes the toned or intensified image we believe to be the silver salt of a complex dye 55 formed by acid oxidation from the hydroquinone dithiosulfate. The reactions taking place with the "mono" and "tetra" forms of the hydroquinone thiosulfuric acid are, we believe, similar to those occurring with the "di" form. The first 60 stage in all the reactions is a bleaching of the image by virtue of formation of the silver salt of the hydroquinone acid employed. The second stage is the darkening of this compound by other substances in solution, the first development of color, probably being due to the formation of a quinhydrone. The third stage is a process occurring simultaneously with the other two, but at a rate varying with the nature of the solution, being the splitting off of silver sulfide from the 65 silver thiosulfate chain.

One of the remarkable properties of our toning baths is that they can be adapted to tone the image immediately after development and before fixing. This is due to the fact that the solubility 70 of the first stage toning product is just less than

that of the silver halides which permits the metallic silver to be converted to silver sulfide under conditions where silver halide remains substantially unattacked.

*Toning.*—Where toning of a print or film, as 5 distinguished from intensification, is desired, the print (or film) after double fixation and a ten-minute wash to assure the removal of all soluble silver compounds, is immersed in a bath such as described above in connection with bromide 10 prints, and containing hydroquinone tetrathiosulfuric acid, and rocked gently until toning is complete. The bath is rich in volatile quinone and should the vapor tend to escape, the tray can be covered with a sheet of glass or Celluloid. The 15 print should then be washed for about 45 minutes to remove the yellow coloration of the whites produced by the quinone. If not completely removed in this way, the yellow color may be eliminated by immersion in a 2% solution of sodium bisulfite 20 at the end of the first ten minutes of washing.

*Intensification.*—The print or film to be intensified is first placed in a new unused bath containing 10-20% of plain hypo for five minutes. It is then washed for ten minutes and placed in 25 a bath such as described above and containing hydroquinone di-thiosulfuric acid, quinone, alum and acid. Two or three minutes are generally required before the reaction is well under way, but when once started can lead to an increase 30 in density of as much as 3 to 5 times in the course of a half hour. The photograph should then be washed for 10-15 minutes.

The colors of the toned image with the hydroquinone thiosulfuric acid toners will vary from 35 brown to a greenish black. The actual color produced varies with the relative quantities of reagents in the bath and with the nature of the particular thiosulfuric acid employed.

We have found that many quinones and substituted quinones can yield thiosulfuric acid derivatives and all form toners with more or less desirable properties. Thus, the mono and dichloroquinones yield thiosulfuric acids conferring a purple tone to silver images. The anthraquinones and the methyl-quinones give thiosulfuric acids, the usefulness of which is somewhat impaired by their sparing solubility, but, nevertheless, they come within the broad scope of our invention, as indeed do any organic compounds 45 containing available sulfur attached to the molecule by another fully oxygenated sulfur atom. No useful purpose would be served by including examples of all of the substituted compounds which are operative in our toning baths, but the following 50 will serve to illustrate the compositions of typical toning baths in which various chloro derivatives may be employed.

|                                               |       |       |
|-----------------------------------------------|-------|-------|
| I. Quinone                                    | g.    | 1.0   |
| Water                                         | c. c. | 100.0 |
| Sulfuric acid                                 | c. c. | .25   |
| and                                           |       |       |
| monochlorohydroquinone monothiosulfuric acid  |       |       |
| in amount to form a saturated solution.       |       | 65    |
| II. Quinone                                   | g.    | 1.0   |
| Water                                         | c. c. | 100.0 |
| Sulfuric acid                                 | c. c. | .25   |
| and                                           |       |       |
| dichlorohydroquinone monothiosulfuric acid in |       | 70    |
| amount to form a saturated solution.          |       |       |
| III. Water                                    | c. c. | * 100 |
| Sulfuric acid                                 | c. c. | 0.25  |
| and                                           |       | 75    |

monochloroquinone monothiosulfuric acid in an amount sufficient to saturate the solution.

Although in the above description we have referred mainly to toning and intensifying baths 5 containing a single quinone or hydroquinone thiosulfuric acid as the essential toning and intensifying constituent, it will be evident that we may employ a plurality of these acids if desired. We may employ, for example, a mixture of hydro- 10 quinone monothiosulfuric acid and hydroquinone dithiosulfuric acid or a mixture of all three of the mono-, di-, and tetra- forms.

As previously indicated, in those cases where 15 a quinone thiosulfuric acid is employed, it is not essential to employ an oxidizing agent due to the fact that the quinone thiosulfuric acid acts as its own oxidizing agent. With the hydroquinone thiosulfuric acids, on the other hand, it is essential to employ an oxidizing agent. Furthermore, 20 these thiosulfuric acids may be used, either in the form of the acid itself or in the form of a soluble salt, such as the potassium salt, it merely being a matter of convenience as to which form is employed.

25 What we claim is:

1. The process of toning and intensifying a developed silver image in a photographic film which comprises treating said image with an aqueous single solution toning and intensifying bath containing as its essential toning and intensifying constituent a quinone thiosulfuric acid selected 30

from the group consisting of quinone monothiosulfuric acid, quinone dithiosulfuric acid and quinone tetrathiosulfuric acid.

2. The process of toning and intensifying a developed silver image in a photographic film which 5 comprises treating said image with an aqueous single solution toning and intensifying bath containing as its essential toning and intensifying constituent quinone monothiosulfuric acid.

3. The process of toning and intensifying a developed silver image in a photographic film which 10 comprises treating said image with an aqueous single solution toning and intensifying bath containing as its essential toning and intensifying constituent quinone dithiosulfuric acid. 15

4. The process of toning and intensifying a developed silver image in a photographic film which 20 comprises treating said image with an aqueous single solution toning and intensifying bath containing as its essential toning and intensifying constituent quinone tetrathiosulfuric acid.

5. The process of toning and intensifying a developed silver image in a photographic film 25 which comprises treating said image with an aqueous single solution toning and intensifying bath containing as its essential toning and intensifying constituent quinone thiosulfuric acid.

KENNETH C. D. HICKMAN. 30  
JOHN C. HECKER.